# EUROPEAN PATENT SPECIFICATION

(11) **EP 3 973 099 B1**
(45) Date of publication and mention of the grant of the patent: **02.07.2025**
(21) Application number: 20728561.0
(22) Date of filing: 20.05.2020
(51) Int. Cl.: D06N 7/00, A47G 27/00, B60N 3/04, D04H 5/00, D04H 5/12, B32B 5/02, B32B 5/26

(54) **PRIMARY CARPET BACKING**
TEPPICHTRÄGER
SUPPORT DE BASE POUR TAPIS

(30) Priority: 22.05.2019 EP 19175831
(43) Date of publication of application: 30.03.2022
(73) Proprietor: Freudenberg Performance Materials LP, Durham, North Carolina 27704 (US)
(72) Inventor: TYLER, Rob, Canton, North Carolina 28716 (US)
(74) Representative: CPW GmbH
(86) International application number: PCT/IB2020/054758
(87) International publication number: WO 2020/234784

(56) References cited:
- WO-A1-2011/069996
- WO-A1-2015/165886
- WO-A1-2016/000869
- WO-A2-03/033801
- GB-A- 1 409 068
- US-A1- 2003 127 768
- US-A1- 2005 148 250
- DATABASE WPI Week 201111, 2011 Derwent World Patents Index; AN 2011-A62246, XP002793101

## Description

The application pertains to a primary carpet backing, a tufted carpet comprising the primary carpet backing and a method for producing such a tufted carpet comprising the primary carpet backing.

In traditional carpet tile productions there are many layers of different material behind the visible pile yarns. The construction behind the pile yarns comprises a primary carpet backing in which the pile yarns are tufted, and the primary carpet backing comprises a precoat to fixate the pile yarns. Below the tufted and precoated primary backing, a traditional carpet tile comprises a layer of polymer, a reinforcement layer, a further layer of polymer and optionally a secondary carpet backing.

This reinforcement layer can be e.g. a fiber glass nonwoven or a scrim, and is responsible for reinforcement in a direction in the plane (x- and y-dimension) of the carpet tile. To transfer occuring forces applied in x- and/or y-direction of the carpet tile to the reinforcement layer, layers of polymer coating are required between the primary carpet backing and the reinforcement layer, and between the secondary carpet backing and the reinforcement layer.

These layers of polymer coating are expensive and carpet tile producers seek to minimize the mass of these two layers of polymer coating, but, a minimum quantity of polymer is required as it is substantial for an adequate bonding between the reinforcement layer and the primary carpet backing and/or between the reinforcement layer and the secondary carpet backing.

In some carpet tiles the reinforcement layer was moved from between the two layers of polymer directly onto the secondary carpet backing, so that it is possible to reduce the two layers of expensive polymer coating to only one layer, and to reduce the total mass of polymer in the carpet tile.

WO 2011/069996 A1 discloses a primary carpet backing comprising a first and a second layer of fibers, wherein both are nonwoven layers of randomly laid fibers and the fibers of the first layer and the second layer copmrise at least two different polymers.

WO 2016/00869 A1 discloses a polyvinyl chloride-free decorative surface comprising a reinforced layer, which is impregnated by a polyvinyl chloride-free paste. Thereby, the polyvinyl chlride-free paste is visible on both sides of the surface covering.

GB 1,409,068 discloses a method for providing a secondary backing to a tufted primary backing. Thereby, the reinforcement of the secondary backing is provided by longitudinal yarns being integral in the knitted structure, which are introduced during and as part of the knitting process.

However, although it is possible to reduce the number of layers of polymer coating by moving the reinforcement layer onto the secondary carpet backing, drawbacks occur like that additional adhesives have to be used to adhere the reinforcement layer onto the secondary carpet backing, and without being bound to theory it is believed that the moving of the reinforcement layer onto the secondary carpet backing has negative consequences for flatness stability (perpendicular to the plane of a carpet tile, z-dimension) like dishing or doming of the carpet tile.

Additionally, if a layer of polymer coating has a high affinity to the primary carpet backing, the polymer coating can be visible on the carpet face, which is known as latex bleeding.

The object of the present application is to provide a material for a primary carpet backing, a tufted carpet comprising the primary carpet backing and a method for producing such a tufted carpet comprising the primary carpet backing, which prevents or at least reduces the aforementioned drawbacks.

The object is reached by a material for a primary carpet backing comprising a structure of at least three layers, wherein a first layer and a third layer comprise a nonwoven layer of fibers, and wherein a second layer comprises a reinforcement layer of fibers and is located between the first and the third layer, , characterized in that the nonwoven layer of fibers of the first layer has an air permeability of at most 8000 l/m²·s, and the nonwoven layer of fibers of the third layer has an air permeability of at least 3500 l/m²·s measured according to ISO 9237:1995, wherein the nonwoven layer of fibers of the first layer has a lower air permeability than the nonwoven layer of fibers of the third layer. Throughout this application, the terms "material for a primary carpet backing" and "primary carpet backing" will be used synonymously.

For clarity reasons, the measuring of the air permeability according to ISO 9237:1995 is performed at a pressure of 200 Pa and a sample having a sample size of 20 cm². Further, the feature that the nonwoven layer of fibers of the first layer has a lower air permeability than the nonwoven layer of fiber of the third layer is also called the "asymmetry of air permeability of the primary carpet backing" for reasons of readability and conciseness.

The fact that the primary carpet backing comprises a reinforcement layer of fibers improves the flatness stability perpendicular to the plane of a carpet tile (z-dimension), like dishing or doming of the carpet tile. The fact that the primary carpet backing comprises a third layer comprising a nonwoven layer of fibers having a minimum air permeability improves penetration of the precoat applied to the tufted primary carpet backing, while the first layer comprising a nonwoven layer of fibers having a reduced air permeability prevents latex bleeding of the precoat to the face of the carpet tile.

For clarity reasons, in the following are clarifications for some terms and phrases which are used during the application.

The term "composite" is to be understood as a material made from two or more constituent materials with significantly different physical or chemical properties that, when combined, produce a material with characteristics different from the individual components.

The phrase "substantially parallel" means that fibers of a unidirectional layer are spaced apart from each other so that the fibers do not contact adjacent fibers of the fibers of the unidirectional layer of fibers.

The terms "spunbonded" and "spun-laid", mean the production of a nonwoven layer of fibers, wherein the fibers are extruded from a spinneret and subsequently laid down on a conveyor belt as a web of filaments and subsequently bonding the web to form a nonwoven layer of fibers, or by a two-step process wherein filaments are spun optionally drawn e. g. using drawing godets or a jet of pressurized air and wound on bobbins, e.g. in the form of multifilament yarns, followed by the steps of unwinding the multifilament yarns and laying the filaments down on a conveyor belt as a web of filaments and bonding the web to form a nonwoven layer of fibers.

The term "carpet face" has to be understood as the side of a carpet which is visible when a carpet is laid on a ground. In the case the carpet is laid on a ground, the side which is not visible is the side which exhibits backstitches of the tufting.

Within the scope of the present application it is understood that the term "fibers" refers to both staple fibers and filaments. Staple fibers are fibers which have a specified, relatively short length in the range of 2 to 200 mm. Filaments are fibers having a length of more than 200 mm. In an embodiment, filaments are fibers with a length of more than 500 mm. In an embodiment, filaments are fibers with a length of more than 1000 mm. Filaments may even be virtually endless, e.g. when formed by continuous extrusion and spinning of a filament through a spinning hole in a spinneret.

Within the scope of the present application "machine direction" is understood to be the direction of production, as it is the largest dimension of the primary carpet backing, which can also be synonymously called x-direction. Further, the "cross machine direction" is the second largest dimension of the primary carpet backing which is in plane with the machine direction and perpendicular to the machine direction, which can be synonymously called y-direction. Out of the plane and perpendicular to the machine direction and the cross machine is the third largest dimension of the primary carpet backing, which is the z-direction.

In an embodiment, the fibers of the nonwoven layer of fibers of the first layer and/or the fibers of the nonwoven layer of fibers of the third layer are filaments.

The primary carpet backing comprises a reinforcement layer of fibers, which can be composed of any suitable material, which is able to reinforce. There are several classes of material available: e.g. high modulus materials, low shrinkage materials and also materials which are resistant to compression.

All classes of materials have their own advantageous properties, for the stability of a primary carpet backing. High modulus materials add the advantageous property that the primary carpet backing has an increased stability against elongation. Low shrinkage materials add the advantageous property that the primary carpet backing has an increased stability against shrinkage, e.g. if temperatures above ambient temperatures impacts the primary carpet backing. Moreover, materials, which are resistant to compression, increase the stability of the primary carpet backing against compression, e.g. stiffness, if e.g. shrinking tufted yarns give a compression force onto the primary carpet backing.

In an embodiment, the fibers of the reinforcement layer of fibers have a tensile modulus of at least 25 GPa. In an embodiment, the fibers of the reinforcement layer of fibers have a tensile modulus of at least 40 GPa. In an embodiment, the fibers of the reinforcement layer of fibers have a tensile modulus of at least 50 GPa. In an embodiment, the fibers of the reinforcement layer of fibers have a tensile modulus of at least 75 GPa.

In an embodiment, the fibers of the reinforcement layer have a linear density of at most 50 tex. In an embodiment, the fibers of the reinforcement layer have a linear density of at most 40 tex. In an embodiment, the fibers of the reinforcement layer have a linear density of at most 30 tex. In an embodiment, the fibers of the reinforcement layer have a linear density of at most 28 tex. In an embodiment, the fibers of the reinforcement layer have a linear density of at most 20 tex. In an embodiment, the fibers of the reinforcement layer have a linear density of at most 15 tex.

In an embodiment of the present application the asymmetry of air permeability of the primary carpet backing is induced by the weight ratio of the nonwoven layer of fibers of the first layer and the nonwoven layer of fibers of the third layer, wherein it is desireable that the nonwoven layer of fibers of the first layer has a higher weight than the nonwoven layer of fibers of the third layer.

The weight ratio of the first layer and the third layer is at least 60:40. In an embodiment, the weight ratio of the first layer and the third layer is at least 70:30. weight ratio of the first layer and the third layer is at least 80:20. weight ratio of the first layer and the third layer is at least 90:10.

In an embodiment, the weight of the first layer comprising a nonwoven layer of fibers is at least 60 g/m². In an embodiment, the weight of the first layer comprising a nonwoven layer of fibers is at least 70 g/m². In an embodiment, the weight of the first layer comprising a nonwoven layer of fibers is at least 80 g/m². In an embodiment, the weight of the first layer comprising a nonwoven layer of fibers is at least 90 g/m². In all cases, the weight is determined accordance with ISO 9073-1.

In an embodiment, the weight of the third layer comprising a nonwoven layer of fibers is at most 40 g/m². In an embodiment, the weight of the third layer comprising a nonwoven layer of fibers is at most 30 g/m². In an embodiment, the weight of the third layer comprising a nonwoven layer of fibers is at most 20 g/m². In an embodiment, the weight of the third layer comprising a nonwoven layer of fibers is at most 10 g/m². The weight is determined in accordance with ISO 9073-1 in all cases.

Due to the higher weight of the nonwoven layer of fibers of the first layer, an increased surface coverage of the fibers in the nonwoven layer of fibers of the first layer and reduced surface coverage of the fibers in the nonwoven layer of fibers of the third layer can occur.

In an embodiment, the first layer comprising a nonwoven layer of fibers has a surface coverage between 1 % and 40 %. In an embodiment, the first layer comprising a nonwoven layer of fibers has a surface coverage between 2 % and 30 %. In an embodiment, the first layer comprising a nonwoven layer of fibers has a surface between 3 % and 25 %. In an embodiment, the first layer comprising a nonwoven layer of fibers has a surface between 5 % and 20 %. The surface coverage A is calculated in the following manner: $A = x ∗ d ;$ with x being the number of filaments per filament layer and d being the diameter of the filaments. The number of filaments per layer x is calculated in the following manner: $x = \frac{N}{L} ;$ wherein N is the number of layers of filaments and L is the total length of filaments per area unit. The quantities N and L are calculated in the following manner: $N = \frac{T}{d} ;$ wherein d is the thickness of the filament in case monofilaments are used and wherein d is the thickness of the filament core in case bicomponent filaments are used. $L = M ∗ t ;$ wherein T is the thickness of the first layer of fibers, M is the area weight of the first layer of fibers and t is the linear density of the filaments. The thickness T is determined in accordance with DIN ISO 9073-2 with a pressure foot of 25 cm² and a pressure of 0.05 kPa.

Without being bound to theory, an increased surface coverage of the fibers in the nonwoven layer of fibers of the first layer can lead to a lower air permeability, thus, inherently to a reduced permeability for fluids e.g. polymer coating and/or precoating.

Otherwise, a reduced surface coverage of the fibers in the nonwoven layer of fibers of the third layer can lead to a higher air permeability, thus, inherently to a higher permeability for fluids e.g. polymer coating and/or precoating.

In an embodiment, the third layer comprising a nonwoven layer of fibers has a surface coverage between 1 % and 40 %. In an embodiment, the third layer comprising a nonwoven layer of fibers has a surface coverage between 2 % and 30 %. In an embodiment, the third layer comprising a nonwoven layer of fibers has a surface between 3 % and 25 %. In an embodiment, the third layer comprising a nonwoven layer of fibers has a surface between 5 % and 20 %.

The asymmetry of air permeability of the primary carpet backing can also be introduced by different average diameters of the fibers comprised in the nonwoven layer of fibers of the first layer and in the nonwoven layer of fibers of the third layer.

In an embodiment, the fibers of the first layer have an average diameter which is smaller than an average diameter of the fibers of the third layer.

In an embodiment, the average diameter of the fibers of the nonwoven layer of fibers of the first layer is at most 50 µm. In an embodiment, the average diameter of the fibers of the nonwoven layer of fibers of the first layer is at most 30 µm. In an embodiment, the average diameter of the fibers of the nonwoven layer of fibers of the first layer is at most 25 µm. In an embodiment, the average diameter of the fibers of the nonwoven layer of fibers of the first layer is at most 20 µm.

In an embodiment, the average diameter of the fibers of the nonwoven layer of fibers of the third layer is at least 30 µm. In an embodiment, the average diameter of the fibers of the nonwoven layer of fibers of the third layer is at least 35 µm. In an embodiment, the average diameter of the fibers of the nonwoven layer of fibers of the third layer is at least 40 µm. In an embodiment, the average diameter of the fibers of the nonwoven layer of fibers of the third layer is at least 50 µm. In an embodiment, the average diameter of the fibers of the nonwoven layer of fibers of the third layer is at least 60 µm.

Without being bound to theory, it is believed that due to the smaller average diameter of the fibers of the nonwoven layer of fibers of the first layer and a higher average diameter of the fibers of the nonwoven layer of fibers of the third layer, differences in surface coverage by fibers in the nonwoven layer of fibers of the first layer and in the nonwoven layer of fibers of the third layer can be provided.

Reducing the average diameter of the fibers e.g. in the nonwoven layer of fibers of the first layer while keeping the weight of the layer constant, the value of length of fibers per square meter (m/m²) of nonwoven layer of fibers of the first layer, i.e. the fiber length per surface area, is increased which can lead to an increased surface coverage of the fibers in the nonwoven layer of fibers of the first layer.

Increasing the average diameter of the fibers e.g. in the nonwoven layer of fibers of the third layer while keeping the weight of the layer constant, the value of length of fibers per square meter (m/m²) of nonwoven layer of fibers of the third layer will be decreased, which can lead to a reduced surface coverage of the fibers in the nonwoven layer of fibers of the third layer.

Accordingly, without being bound to theory it is believed that by combining a higher weight of a layer of fibers and a smaller average diameter of the fibers of a layer, e.g. in the nonwoven layer of fibers of the first layer, can synergistically support the effect of a lower air permeability and a lower permeability for fluids e.g. polymer coating and/or precoating.

Otherwise, by combining a lower weight of a layer of fibers and a higher average diameter of the fibers of a layer, e.g. of the nonwoven layer of fibers of the third layer, can synergistically support the effect of a higher air permeability and a higher permeability for fluids e.g. polymer coating and/or precoating.

The nonwoven layer of fibers of the first layer and/or the nonwoven layer of fibers of the third layer can comprise mono-component fibers, two types of mono-component fibers and/or bicomponent fibers.

The nonwoven layer of fibers of the first layer and/or the nonwoven layer of fibers of the third layer can be made by any suitable process, such as a spun-laid process, air-laid process, wet-laid process, melt-blown process, or a carding process.

In an embodiment, the nonwoven layer of fibers of the first layer and/or the nonwoven layer of fibers of the third layer are made by a spun-laid process, wherein the fibers are made from a thermoplastic polymeric material. In the spun-laid process, bonding of the fibers of the nonwoven layer of fibers of the first layer and/or of the nonwoven layer of fibers of the third layer can be conducted by any suitable process, including hydro entanglement, needling, chemical bonding, calendaring, ultrasonic bonding, and other thermal bonding methods e.g. hot air bonding.

In an embodiment, the nonwoven layer of fibers of the first layer and/or the nonwoven layer of fibers of the third layer comprises two types of mono component fibers which comprise two chemically different thermoplastic polymeric materials, wherein two types of mono-component fibers differ in melting temperature by at least of 10°C. In an embodiment, the difference in melting temperature between the two thermoplastic polymeric materials is 20°C. In an embodiment, the difference in melting temperature between the two thermoplastic polymeric materials is 30°C. In an embodiment, the difference in melting temperature between the two thermoplastic polymeric materials is 50°C.

In an embodiment, the fibers of the nonwoven layers of fibers of the first layer and/or the fibers of the nonwoven layer fibers of the third layer are bicomponent fibers of the concentric or eccentric core/sheath model, side-by-side model, segmented pie model or island-in-the-sea model.

In an embodiment, the fibers of the nonwoven layer of fibers of the first layer and/or the fibers of the nonwoven layer fibers of the third layer are bicomponent fibers of the concentric core/sheath model, wherein the fibers are made of the same class of thermoplastic polymeric material or of chemically different thermoplastic polymeric materials.

Within the scope of the application, the same class of thermoplastic material means that same monomeric units of the polymer can be used, but the thermoplastic polymeric material can be different by a different polymer chain length, by a different density of the thermoplastic polymeric material or by a different orientation of the monomeric units, which can be isotactic, syndiotactic or atactic.

The core of the bicomponent fiber can comprise a thermoplastic polymeric material, which has a higher melting temperature as the thermoplastic polymeric material of the sheath. The melting temperature of the thermoplastic polymeric material of the core and the thermoplastic polymeric material of the sheath may differ by at least 10°C. The melting temperature of the thermoplastic polymeric material of the core and the thermoplastic polymeric material of the sheath may differ by at least 20°C. The melting temperature of the thermoplastic polymeric material of the core and the thermoplastic polymeric material of the sheath may differ by at least 30°C. The melting temperature of the thermoplastic polymeric material of the core and the thermoplastic polymeric material of the sheath may differ by at least 50°C.

The thermoplastic polymeric material of the fibers of the nonwoven layers of fibers of the first layer and/or the fibers of the nonwoven layer fibers of the third layer can be selected from a group comprising polyolefins such as polyethylene (PE) and polypropylene (PP), polyesters such as polyethylene terephthalate (PET), polytrimethylene terephthalate (PTT), polybutylene terephthalate (PBT), polyethylene naphthalate (PEN), polyetylene-1,2-furandicaboxylate (PEF), and poly lactic acid (PLA), polyamides such as polyamide 6,6 (PA6,6) and polyamide 6 (PA6), and copolymers and/or blends thereof.

In an embodiment, the fibers of the nonwoven layer of fibers of the first layer and/or the fibers of the nonwoven layer fibers of the third layer comprise at least 50 wt.-% of a thermoplastic material. In an embodiment, the fibers of the nonwoven layer of fibers of the first layer and/or the fibers of the nonwoven layer fibers of the third layer comprise at least 75 wt.-% of a thermoplastic material. In an embodiment, the fibers of the nonwoven layer of fibers of the first layer and/or the fibers of the nonwoven layer fibers of the third layer comprise at least 85 wt.-% of a thermoplastic material. In an embodiment, the fibers of the nonwoven layer of fibers of the first layer and/or the fibers of the nonwoven layer fibers of the third layer comprise at least 95 wt.-% of a thermoplastic material. In an embodiment, the fibers of the nonwoven layer of fibers of the first layer and/or the fibers of the nonwoven layer fibers of the third layer comprise at least 97 wt.-% of a thermoplastic material.

Thereby, the thermoplastic polymeric material can comprise additives such as flame retardents, coloring agents, fillers, fungicides, and/or anti-bacterial agents.

In an embodiment, the reinforcement layer comprised in the primary carpet backing can be a nonwoven fabric, a woven fabric, a laid scrim, a woven scrim, a unidirectional layer of fibers, or a knitted fabric.

In an embodiment, the reinforcement layer of the primary carpet backing is a laid scrim, a woven scrim or an unidirectional layer of fibers, wherein the fibers of the unidirectional layer of fibers are aligned substantially parallel to each other in the machine direction.

In an embodiment, the fibers of the unidirectional layer of fibers, which have huge length in view of width and height (e.g. filaments), are spaced apart from each other at a constant distance over the entire length of the unidirectional layer of fibers. Within the scope of this application, a constant distance may mean that the shortest distance between two threads does not differ by more than 2 millimeters. Within the scope of this application, a constant distance may mean that the shortest distance between two threads does not differ by more than 1 millimeters. Within the scope of this application, a constant distance may mean that the shortest distance between two threads does not differ by more than 0.5 millimeters.

As it is well known to the person skilled in the art, a scrim, no matter if laid or woven, is an open lattice structure composed of at least two sets of parallel threads, wherein the first group of parallel threads is oriented at an angle, generally at a 90° angle, to the second group of parallel threads. The first group of parallel threads may be connected to the second group of parallel threads by chemical bonding to form a laid scrim or the first group of parallel threads may be interwoven with the second group of parallel threads to form a woven scrim. In an embodiment, the openings in the scrim have at least one dimension in the plane of the scrim being at least 1 mm. In an embodiment, the openings in the scrim have at least one dimension in the plane of the scrim being at least 2 mm. In an embodiment, the openings in the scrim have at least one dimension in the plane of the scrim being at least 5 mm.

In an embodiment, the reinforcement layer of fibers comprised in the primary carpet backing comprises high modulus fibers is composed of a material selected from a group comprising glass, carbon, basalt, high modulus low shrinkage (HMLS) polyester, mineral material, aramid such as para aramid (PPTA) and meta aramid (MPTA), and ultra-high molecular weight polyethylene (UHMWPE).

In an embodiment, nonwoven layer of fibers of the first layer of the primary carpet backing can have an air permeability of at most 7000 l/m²·s. In an embodiment, nonwoven layer of fibers of the first layer of the primary carpet backing can have an air permeability of at most 6000 l/m²·s. In an embodiment, nonwoven layer of fibers of the first layer of the primary carpet backing can have an air permeability of at most 5000 l/m²·s. In an embodiment, nonwoven layer of fibers of the first layer of the primary carpet backing can have an air permeability of at most 4000 l/m²·s. In an embodiment, nonwoven layer of fibers of the first layer of the primary carpet backing can have an air permeability of at most 3000 l/m²·s. In an embodiment, nonwoven layer of fibers of the first layer of the primary carpet backing can have an air permeability of at most 2000 l/m²·s. In an embodiment, nonwoven layer of fibers of the first layer of the primary carpet backing can have an air permeability of at most 1000 l/m²·s. The air permeability is measured according to ISO 9237:1995 in all cases.

In an embodiment, the nonwoven layer of fibers of the second layer and/or third layer of the primary carpet backing can have an air permeability of at least 5000 l/m²·s. In an embodiment, the nonwoven layer of fibers of the second layer and/or third layer of the primary carpet backing can have an air permeability of at least 65000 l/m²·s. In an embodiment, the nonwoven layer of fibers of the second layer and/or third layer of the primary carpet backing can have an air permeability of at least 8000 l/m²·s. In an embodiment, the nonwoven layer of fibers of the second layer and/or third layer of the primary carpet backing can have an air permeability of at least 9500 l/m²·s. In an embodiment, the nonwoven layer of fibers of the second layer and/or third layer of the primary carpet backing can have an air permeability of at least 12000 l/m²·s. The air permeability is measured according to ISO 9237:1995 in all cases.

The object is also solved by a tufted carpet comprising a primary carpet backing according to any of the aforementioned embodiments, pile yarns tufted into the primary carpet backing, optionally a secondary carpet backing, adjoining on the side of the primary carpet backing which is not the carpet face, and/or optionally a precoat and/or a polymer coat.

Without being bound to theory, it is believed that due to asymmetry of air permeability of the primary carpet backing the precoat and/or the polymer coat is able to diffuse through the third layer and the second layer having a higher air permeability. Further, it is believed that due to the lower air permeability of the first layer of the primary carpet backing, the first layer acts as a barrier layer and does not permit or at least limits the precoat and/or polymer coat to diffuse through, which prevents or at least reduces latex bleeding.

In an embodiment, the secondary carpet backing can comprise a reinforcement layer of fibers which can be composed of any suitable material which is able to reinforce. There are a few classes of material available: e.g. high modulus materials, low shrinkage materials and also materials which are resistant to compression.

Without being bound to theory, it is believed that positioning of the secondary carpet backing directly next to the primary carpet backing will further reduce dishing and doming of the tufted carpet.

The reinforcement layer of the secondary carpet backing can be a nonwoven fabric, a woven fabric, a scrim, a unidirectional layer of fibers, or a knitted fabric.

In an embodiment, the reinforcement layer of the secondary carpet backing is a laid scrim, a woven scrim, or a unidirectional layer of fibers, wherein the fibers of the unidirectional layer of fibers are aligned substantially parallel to each other in the machine direction. Thereby, the fibers of the unidirectional layer of the secondary carpet backing are spaced apart from each other so that the fibers do not contact adjacent fibers of the unidirectional layer of fibers of the secondary carpet backing.

In an embodiment, the fibers of the unidirectional layer of fibers are spaced apart from each other at a constant distance over the entire length of the unidirectional layer of fibers.

In an embodiment, the reinforcement layer of the secondary carpet backing is made of high modulus fibers. The fibers may be composed of a material selected from a group comprising glass, carbon, basalt, high modulus low shrinkage (HMLS) polyester, mineral material, aramid such as para aramid (PPTA) and meta aramid (MPTA), ultra-high molecular weight polyethylene (UHMWPE).

In an embodiment the secondary carpet backing comprises a composite of at least three layers comprising two nonwoven layers of fibers and the reinforcement layer is located between the two nonwoven layers of fibers, wherein the secondary carpet backing has an air permeability of at least 1000 l/m²·s. In an embodiment the secondary carpet backing comprises a composite of at least three layers comprising two nonwoven layers of fibers and the reinforcement layer is located between the two nonwoven layers of fibers, wherein the secondary carpet backing has an air permeability of at least 3000 l/m²·s. In an embodiment the secondary carpet backing comprises a composite of at least three layers comprising two nonwoven layers of fibers and the reinforcement layer is located between the two nonwoven layers of fibers, wherein the secondary carpet backing has an air permeability of at least 5000 l/m²·s. In an embodiment the secondary carpet backing comprises a composite of at least three layers comprising two nonwoven layers of fibers and the reinforcement layer is located between the two nonwoven layers of fibers, wherein the secondary carpet backing has an air permeability of at least 7000 l/m²·s. In an embodiment the secondary carpet backing comprises a composite of at least three layers comprising two nonwoven layers of fibers and the reinforcement layer is located between the two nonwoven layers of fibers, wherein the secondary carpet backing has an air permeability of at least 9000 l/m²·s. In an embodiment the secondary carpet backing comprises a composite of at least three layers comprising two nonwoven layers of fibers and the reinforcement layer is located between the two nonwoven layers of fibers, wherein the secondary carpet backing has an air permeability of at least 10500 l/m²·s. In an embodiment the secondary carpet backing comprises a composite of at least three layers comprising two nonwoven layers of fibers and the reinforcement layer is located between the two nonwoven layers of fibers, wherein the secondary carpet backing has an air permeability of at least 12000 l/m²·s. The air permeability being measured according to ISO 9237:1995.

One or both of the nonwoven layers of fibers of the secondary carpet backing can have an average weight of at most 50 g/m². One or both of the nonwoven layers of fibers of the secondary carpet backing can have an average weight of at most 30 g/m². One or both of the nonwoven layers of fibers of the secondary carpet backing can have an average weight of at most 30 g/m². One or both of the nonwoven layers of fibers of the secondary carpet backing can have an average weight of at most 20 g/m². One or both of the nonwoven layers of fibers of the secondary carpet backing can have an average weight of at most 10 g/m². One or both of the nonwoven layers of fibers of the secondary carpet backing can have an average weight of at most 7 g/m².

In an embodiment, the average diameter of the fibers of one or both of the two nonwoven layers of fibers of the secondary carpet backing is at least 30 µm. In an embodiment, the average diameter of the fibers of one or both of the two nonwoven layers of fibers of the secondary carpet backing is at least 35 µm. In an embodiment, the average diameter of the fibers of one or both of the two nonwoven layers of fibers of the secondary carpet backing is at least 40 µm. In an embodiment, the average diameter of the fibers of one or both of the two nonwoven layers of fibers of the secondary carpet backing is at least 50 µm. In an embodiment, the average diameter of the fibers of one or both of the two nonwoven layers of fibers of the secondary carpet backing is at least 60 µm.

One or both of the two nonwoven layers of fibers of the secondary carpet backing can comprise mono-component fibers, two types of mono-component fibers and/or bicomponent fibers.

One or both nonwoven layer of fibers of the secondary carpet backing can be made by various processes: a spun-laid process, air-laid process, wet-laid process, melt-blown process, or a carding process.

In an embodiment, one or both nonwoven layers of fibers of the secondary carpet backing are made by a spun-laid process, wherein the fibers are made from a thermoplastic polymeric material. In the spun-laid process, bonding of the fibers of the nonwoven layer of fibers of the first layer and/or of the nonwoven layer of fibers of the third layer can be conducted by any suitable process, including calendaring, hydro entanglement, needling, ultrasonic bonding, chemical bonding, and other thermal bonding method e.g. hot air bonding.

In an embodiment, one or both nonwoven layers of fibers of the secondary carpet backing comprises two types of mono component fibers which comprises two chemically different thermoplastic polymeric materials, wherein the melting temperature of the different thermoplastic polymeric materials differs by at least by 10°C. In an embodiment, the melting temperature of the different thermoplastic polymeric materials differs by at least by 20°C. In an embodiment, the melting temperature of the different thermoplastic polymeric materials differs by at least by 30°C. In an embodiment, the melting temperature of the different thermoplastic polymeric materials differs by at least by 50°C.

In an embodiment, the fibers of one or both of the nonwoven layers of fibers of the secondary carpet backing are bicomponent fibers of the concentric or eccentric core/sheath model, side-by-side model, segmented pie model or island-in-the-sea model.

In an embodiment, the fibers of one or both of the nonwoven layers of fibers of the secondary carpet backing are bicomponent fibers of the concentric core/sheath model, wherein the fibers are made of the same class of thermoplastic polymeric material or chemically different thermoplastic polymeric materials.

The sheath of the bicomponent fibers of one or both nonwoven layers of fibers of the secondary carpet backing can comprise a thermoplastic polymeric material, which has a higher melting temperature as the thermoplastic polymeric material of the core. The melting temperature of the thermoplastic polymeric material of the sheath and the thermoplastic polymeric material of the core may differ by at least 10°C. The melting temperature of the thermoplastic polymeric material of the sheath and the thermoplastic polymeric material of the core may differ by at least 20°C. The melting temperature of the thermoplastic polymeric material of the sheath and the thermoplastic polymeric material of the core may differ by at least 30°C. The melting temperature of the thermoplastic polymeric material of the sheath and the thermoplastic polymeric material of the core may differ by at least 50°C.

The thermoplastic polymeric material of the fibers of both nonwoven layers of fibers of the secondary carpet backing can be selected from a group comprising polyolefins such as polyethylene (PE) and polypropylene (PP), polyesters such as polyethylene terephthalate (PET) polytrimethylene terephthalate (PTT), polybutylene terephthalate (PBT), polyethylene naphthalate (PEN) polyetylene-1,2-furandicaboxylate (PEF),and poly lactic acid (PLA), polyamides such as polyamide 6,6 (PA6,6) and polyamide 6 (PA6), and copolymers and/or blends thereof.

In an embodiment, the fibers of both nonwoven layer of fibers comprise at least 50 wt.-% of a thermoplastic material. In an embodiment, the fibers of both nonwoven layer of fibers comprise at least 75 wt.-% of a thermoplastic material. In an embodiment, the fibers of both nonwoven layer of fibers comprise at least 85 wt.-% of a thermoplastic material. In an embodiment, the fibers of both nonwoven layer of fibers comprise at least 95 wt.-% of a thermoplastic material. In an embodiment, the fibers of both nonwoven layer of fibers comprise at least 97 wt.-% of a thermoplastic material.

Thereby, the thermoplastic polymeric material can comprise additives such as flame retardents, coloring agents, filler, fungicides, and/or anti-bacterial agents.

The tufted carpet according to the application can be manufactured by tufting a primary carpet backing, supplying a secondary carpet backing to the tufted primary carpet backing, on the side of the tufted primary carpet backing which is not the carpet face, and supplying a precoat into and/or onto the secondary backing from the side of the secondary carpet backing which is not facing the primary carpet backing, and optionally a polymer coating.

The primary carpet backing can be a composite being tufted, but it is also possible that the layers of the primary carpet backing are individual layers, which are adjoining each other, thus, the layers of the primary carpet backing are supplied individually to the tufting machine.

In an embodiment, the layers of the primary carpet backing are tufted as a composite.

## Claims

1. A material for a primary carpet backing comprising a structure of at least three layers, wherein a first layer and a third layer comprise a nonwoven layer of fibers, and wherein a second layer comprises a reinforcement layer of fibers and is located between the first and the third layer, **characterized in that** the nonwoven layer of fibers of the first layer has an air permeability of at most 8000 I/m²·s, and the nonwoven layer of fibers of the third layer has an air permeability of at least 3500 l/m²·s measured according to ISO 9237:1995, wherein the nonwoven layer of fibers of the first layer has a lower air permeability than the nonwoven layer of fibers of the third layer.

2. The material according to claim 1, **characterized in that** a weight ratio of the first layer and the second layer is of at least 60:40, preferably of at least 70:30, even more preferably of at least 80:20, and most preferably of at least 90:10.

3. The material according to any of the preceding claims, **characterized in that** the fibers of the first layer have an average diameter, which is smaller than an average diameter of the fibers of the third layer.

4. The material according to claim 3, **characterized in that** the fibers of the first layer have an average diameter of at most 50 µm, preferably of at most 40 µm, more preferably of at most 30 µm, even more preferably of at most 25 µm, and most preferably of at most 20 µm and/or the fibers of the third layer have an average diameter of at least 30 µm, preferably of at least 35 µm, more preferably of at least 40 µm, even more preferably of at least 50 µm, and most preferably of at least 60 µm.

5. The material according to any of claims 1 to 4, **characterized in that** nonwoven layer of fibers of the first layer and/or the nonwoven layer of fibers of the third layer comprise mono-component fibers, two types of mono-component fibers and/or bicomponent fibers.

6. The material according to any of claims 1 to 5, **characterized in that** the nonwoven layer of fibers of the first layer and/or the nonwoven layer of fibers of the third layer are made by a spun-laid process, wherein the fibers are made from a thermoplastic polymeric material.

7. The material according to any of the preceding claims, **characterized in that** the reinforcement layer is a laid scrim, a woven scrim or a unidirectional layer of fibers, wherein the fibers of the unidirectional layer of fibers are aligned substantially parallel to each other in the machine direction.

8. The material according to any of the preceding claims, **characterized in that** the reinforcement layer is made of high modulus fibers or filaments composed of a material, preferably selected from a group comprising glass, carbon, basalt, stone wool, high modulus low shrinkage polyester, mineral material, aramid such as para aramid and meta aramid, ultra high molecular weight polyethylene.

9. The material according to any of the preceding claims, **characterized in that** the nonwoven layer of fibers of the first layer has an air permeability of at most 7000 I/m²·s, preferably of at most 6000 I/m²·s, more preferably of at most 5000 I/m²·s, even more preferably of at most 4000 I/m²·s, even more preferably of at most 3000 l/m²·s, even more preferably of at most 2000 l/m²·s, and most preferably of at most 1000 l/m²·s, measured according to ISO 9237:1995.

10. The material according to any of the preceding claims, **characterized in that** the air permeability of the nonwoven layer of fibers of the third layer is of at least 5000 I/m²·s, more preferably of at least 6500 L/m²·s, even more preferably of at least 8000 I/m²·s, even more preferably of at least 9500 l/m²·s, and most preferably of at least 12000 l/m²·s, measured according to ISO 9237.

11. A tufted carpet comprising material according to any of the preceding claims, pile yarns tufted into the primary carpet backing, optionally a secondary carpet backing, adjoining on the side of the primary carpet backing which is not the carpet face, and/or optionally a precoat and/or a polymer coat.

12. The tufted carpet according to claim 11, **characterized in that** the secondary carpet backing comprises a reinforcement layer.

13. The tufted carpet according to claim 12, **characterized in that** the secondary carpet backing comprises a composite of at least three layers comprising two nonwoven layers of fibers and the reinforcement layer is located between the two spunbonded nonwoven layers of fibers, wherein the secondary carpet backing has an air permeability of at least 1000 I/m²·s, measured according to ISO 9237:1995.

14. The tufted carpet according to claim 13, **characterized in that** the fibers of the two nonwoven layer of fibers of the secondary carpet backing comprises have an average diameter of at least 30 µm, preferably of at least 35 µm, more preferably of at least 40 µm, even more preferably of at least 50 µm, and most preferably of at least 60 µm.

15. A process of producing a tufted carpet according to any of the claims 11 to 14 by tufting a primary carpet backing, supplying a secondary carpet backing to the tufted primary carpet backing, on the side of the tufted primary carpet backing which is not the carpet face, and supplying a precoat into and/or onto the secondary backing from the side of the secondary carpet backing which is not facing the primary carpet backing, and optionally a polymer coating.

## Patentansprüche

1. Material für einen primären Teppichträger, das eine Struktur aus mindestens drei Schichten umfasst, wobei eine erste Schicht und eine dritte Schicht eine Vliesfaserschicht umfassen, und wobei eine zweite Schicht eine Verstärkungsfaserschicht umfasst und sich zwischen der ersten und der dritten Schicht befindet, **dadurch gekennzeichnet, dass** die Vliesfaserschicht der ersten Schicht eine Luftdurchlässigkeit von höchstens 8000 l/m²·s aufweist, und die Vliesfaserschicht der dritten Schicht eine Luftdurchlässigkeit von mindestens 3500 l/m²·s, gemessen nach ISO 9237:1995, aufweist, wobei die Vliesfaserschicht der ersten Schicht eine geringere Luftdurchlässigkeit aufweist als die Vliesfaserschicht der dritten Schicht.

2. Material nach Anspruch 1, **dadurch gekennzeichnet, dass** ein Gewichtsverhältnis zwischen der ersten Schicht und der zweiten Schicht mindestens 60:40, vorzugsweise mindestens 70:30, noch bevorzugter mindestens 80:20 und besonders bevorzugt mindestens 90:10 beträgt.

3. Material nach einem der vorstehenden Ansprüche, **dadurch gekennzeichnet, dass** die Fasern der ersten Schicht einen mittleren Durchmesser aufweisen, der kleiner ist als ein mittlerer Durchmesser der Fasern der dritten Schicht.

4. Material nach Anspruch 3, **dadurch gekennzeichnet, dass** die Fasern der ersten Schicht einen mittleren Durchmesser von höchstens 50 µm, vorzugsweise von höchstens 40 µm, bevorzugter von höchstens 30 µm, noch bevorzugter von höchstens 25 µm und besonders bevorzugt von höchstens 20 µm aufweisen und/oder die Fasern der dritten Schicht einen mittleren Durchmesser von mindestens 30 µm, vorzugsweise von mindestens 35 µm, bevorzugter von mindestens 40 µm, noch bevorzugter von mindestens 50 µm und besonders bevorzugt von mindestens 60 µm aufweisen.

5. Material nach einem der Ansprüche 1 bis 4, **dadurch gekennzeichnet, dass** die Vliesfaserschicht der ersten Schicht und/oder die Vliesfaserschicht der dritten Schicht Einkomponentenfasern, zwei Arten von Einkomponentenfasern und/oder Bikomponentenfasern umfassen.

6. Material nach einem der Ansprüche 1 bis 5, **dadurch gekennzeichnet, dass** die Vliesfaserschicht der ersten Schicht und/oder die Vliesfaserschicht der dritten Schicht durch ein Spinnvliesverfahren hergestellt sind, wobei die Fasern aus einem thermoplastischen Polymermaterial hergestellt sind.

7. Material nach einem der vorstehenden Ansprüche, **dadurch gekennzeichnet, dass** die Verstärkungsschicht ein gelegtes Gitter, ein gewebtes Gitter oder eine unidirektionale Faserschicht ist, wobei die Fasern der unidirektionalen Faserschicht im Wesentlichen parallel zueinander in der Maschinenrichtung ausgerichtet sind.

8. Material nach einem der vorstehenden Ansprüche, **dadurch gekennzeichnet, dass** die Verstärkungsschicht aus hochmoduligen Fasern oder Filamenten hergestellt ist, die aus einem Material bestehen, das vorzugsweise aus einer Gruppe ausgewählt ist, die Glas, Kohlenstoff, Basalt, Steinwolle, hochmoduliges Polyester mit geringer Schrumpfung, mineralisches Material, Aramid, wie beispielsweise Para-Aramid und Meta-Aramid, Polyethylen mit ultrahohem Molekulargewicht umfasst.

9. Material nach einem der vorstehenden Ansprüche, **dadurch gekennzeichnet, dass** die Vliesfaserschicht der ersten Schicht eine Luftdurchlässigkeit von höchstens 7000 l/m²·s, vorzugsweise von höchstens 6000 l/m²·s, bevorzugter von höchstens 5000 l/m²·s, noch bevorzugter von höchstens 4000 l/m²·s, noch bevorzugter von höchstens 3000 l/m²·s, noch bevorzugter von höchstens 2000 l/m²·s und besonders bevorzugt von höchstens 1000 l/m²·s, gemessen nach ISO 9237:1995, aufweist.

10. Material nach einem der vorstehenden Ansprüche, **dadurch gekennzeichnet, dass** die Luftdurchlässigkeit der Vliesfaserschicht der dritten Schicht mindestens 5000 l/m²·s, bevorzugter mindestens 6500 L/m²·s, noch bevorzugter mindestens 8000 l/m²·s, noch bevorzugter mindestens 9500 l/m²·s und besonders bevorzugt mindestens 12000 l/m²·s beträgt, gemessen nach ISO 9237.

11. Tuftingteppich, umfassend ein Material nach einem der vorstehenden Ansprüche, in den primären Teppichträger getuftete Florfäden, optional einen sekundären Teppichträger, der an die Seite des primären Teppichträgers angrenzt, die nicht die Teppichoberfläche ist, und/oder optional eine Vorbeschichtung und/oder eine Polymerbeschichtung.

12. Tuftingteppich nach Anspruch 11, **dadurch gekennzeichnet, dass** der sekundäre Teppichträger eine Verstärkungsschicht umfasst.

13. Tuftingteppich nach Anspruch 12, **dadurch gekennzeichnet, dass** der sekundäre Teppichträger einen Verbund aus mindestens drei Schichten umfasst, der zwei Vliesfaserschichten umfasst, und dass die Verstärkungsschicht sich zwischen den beiden Spinnvliesfaserschichten befindet, wobei der sekundäre Teppichträger eine Luftdurchlässigkeit von mindestens 1000 l/m²·s, gemessen nach ISO 9237:1995, aufweist.

14. Tuftingteppich nach Anspruch 13, **dadurch gekennzeichnet, dass** die Fasern der beiden Vliesfaserschichten des sekundären Teppichträgers einen mittleren Durchmesser von mindestens 30 µm, vorzugsweise von mindestens 35 µm, bevorzugter von mindestens 40 µm, noch bevorzugter von mindestens 50 µm und besonders bevorzugt von mindestens 60 µm aufweisen.

15. Verfahren zur Herstellung eines Tuftingteppichs nach einem der Ansprüche 11 bis 14 durch Tuften eines primären Teppichträgers, Zuführen eines sekundären Teppichträgers zu dem getufteten primären Teppichträger auf der Seite des getufteten primären Teppichträgers, die nicht die Teppichoberfläche ist, und Zuführen einer Vorbeschichtung in und/oder auf den sekundären Rücken von der Seite des sekundären Teppichträgers, die nicht dem primären Teppichträger zugewandt ist, und optional einer Polymerbeschichtung.

## Revendications

1. Matériau pour un endos de tapis primaire comprenant une structure d'au moins trois couches, dans lequel une première couche et une troisième couche comprennent une couche de fibres non tissée, et dans lequel une deuxième couche comprend une couche de fibres de renfort et est située entre la première et la troisième couche, **caractérisé en ce que** la couche de fibres non tissée de la première couche présente une perméabilité à l'air d'au plus 8000 l/m²·s, et la couche de fibres non tissée de la troisième couche présente une perméabilité à l'air d'au moins 3500 l/m²·s mesurée selon la norme ISO 9237:1995, dans lequel la couche de fibres non tissée de la première couche présente une perméabilité à l'air inférieure à la couche de fibres non tissée de la troisième couche.

2. Matériau selon la revendication 1, **caractérisé en ce qu'**un rapport pondéral de la première couche et de la deuxième couche est d'au moins 60:40, de préférence d'au moins 70:30, de manière davantage préférée d'au moins 80:20, et de manière préférée entre toutes d'au moins 90:10.

3. Matériau selon l'une quelconque des revendications précédentes, **caractérisé en ce que** les fibres de la première couche présentent un diamètre moyen, qui est inférieur à un diamètre moyen des fibres de la troisième couche.

4. Matériau selon la revendication 3, **caractérisé en ce que** les fibres de la première couche présentent un diamètre moyen d'au plus 50 µm, de préférence d'au plus 40 µm, de manière davantage préférée d'au plus 30 µm, de manière encore davantage préférée d'au plus 25 µm, et de manière préférée entre toutes d'au plus 20 µm et/ou les fibres de la troisième couche présentent un diamètre moyen d'au moins 30 µm, de préférence d'au moins 35 µm, de manière davantage préférée d'au moins 40 µm, de manière encore davantage préférée d'au moins 50 µm, et de manière préférée entre toutes d'au moins 60 µm.

5. Matériau selon l'une quelconque des revendications 1 à 4, **caractérisé en ce que** la couche de fibres non tissée de la première couche et/ou la couche de fibres non tissée de la troisième couche comprennent des fibres monocomposantes, deux types de fibres monocomposantes et/ou des fibres bicomposantes.

6. Matériau selon l'une quelconque des revendications 1 à 5, **caractérisé en ce que** la couche de fibres non tissée de la première couche et/ou la couche de fibres non tissée de la troisième couche sont réalisées par un procédé filé-lié, dans lequel les fibres sont constituées d'un matériau polymère thermoplastique.

7. Matériau selon l'une quelconque des revendications précédentes, **caractérisé en ce que** la couche de renfort est une grille posée, une grille tissée ou une couche unidirectionnelle de fibres, dans lequel les fibres de la couche unidirectionnelle de fibres sont alignées de manière sensiblement parallèle les unes aux autres dans le sens de la machine.

8. Matériau selon l'une quelconque des revendications précédentes, **caractérisé en ce que** la couche de renfort est en fibres ou en filaments à module élevé composés d'un matériau, de préférence sélectionné parmi un groupe comprenant le verre, le carbone, le basalte, la laine de roche, un polyester à module élevé et à faible rétrécissement, un matériau minéral, un aramide tel que le para-aramide et le méta-aramide, un polyéthylène à poids moléculaire ultra élevé.

9. Matériau selon l'une quelconque des revendications précédentes, **caractérisé en ce que** la couche de fibres non tissée de la première couche présente une perméabilité à l'air d'au plus 7000 l/m²·s, de préférence d'au plus 6000 l/m²·s, de manière davantage préférée d'au plus 5000 I/m²·s, de manière encore davantage préférée d'au plus 4000 l/m²·s, de manière encore davantage préférée d'au plus 3000 I/m²·s, de manière encore davantage préférée d'au plus 2000 l/m²·s, et de manière préférée entre toutes d'au plus 1000 l/m²·s, mesurée selon la norme ISO 9237:1995.

10. Matériau selon l'une quelconque des revendications précédentes, **caractérisé en ce que** la perméabilité à l'air de la couche de fibres non tissée de la troisième couche est d'au moins 5000 l/m²·s, de manière davantage préférée d'au moins 6500 l/m²·s, de manière encore davantage préférée d'au moins 8000 l/m²·s, de manière encore davantage préférée d'au moins 9500 l/m²·s, et de manière préférée entre toutes d'au moins 12 000 l/m²·s, mesurée selon la norme ISO 9237.

11. Tapis tufté comprenant un matériau selon l'une quelconque des revendications précédentes, des fils de velours tuftés dans l'endos de tapis primaire, facultativement dans un endos de tapis secondaire, jouxtant le côté de l'endos de tapis primaire qui n'est pas la face de tapis, et/ou facultativement une précouche et/ou un revêtement polymère.

12. Tapis tufté selon la revendication 11, **caractérisé en ce que** l'endos de tapis secondaire comprend une couche de renfort.

13. Tapis tufté selon la revendication 12, **caractérisé en ce que** l'endos de tapis secondaire comprend un composite d'au moins trois couches comprenant deux couches de fibres non tissées et la couche de renfort est située entre les deux couches de fibres non tissées filées-liées, dans lequel l'endos de tapis secondaire présente une perméabilité à l'air d'au moins 1000 l/m²·s, mesurée selon la norme ISO 9237:1995.

14. Tapis tufté selon la revendication 13, **caractérisé en ce que** les fibres des deux couches de fibres non tissées de l'endos de tapis secondaire comprennent un diamètre moyen d'au moins 30 µm, de préférence d'au moins 35 µm, de manière davantage préférée d'au moins 40 µm, de manière encore davantage préférée d'au moins 50 µm, et de manière préférée entre toutes d'au moins 60 µm.

15. Procédé de production d'un tapis tufté selon l'une quelconque des revendications 11 à 14 par tuftage d'un endos de tapis primaire, une fourniture d'un endos de tapis secondaire à l'endos de tapis primaire tufté, sur le côté de l'endos de tapis primaire tufté qui n'est pas la face de tapis, et une fourniture d'une précouche dans et/ou sur l'endos secondaire à partir du côté de l'endos de tapis secondaire qui ne fait pas face à l'endos de tapis primaire, et facultativement d'un revêtement polymère.
